

## UNITED STATES PATENT OFFICE.

RICHARD WALTER, OF DUSSELDORF, GERMANY.

## METHOD OF MAKING ALLOYS.

No Drawing.

Application filed June 28, 1920. Serial No. 392,501.

*To all whom it may concern:*

Be it known that I, RICHARD WALTER, residing at Dusseldorf, Germany, a citizen of the German Empire, have invented certain new and useful Improvements in Methods of Making Alloys (for which I filed applications in Austria Mar. 20, 1918, and in Germany May 28, 1919), of which the following is a specification.

- 10 This invention relates to improvements in making alloys and more particularly to a process for alloying metals of the iron and chromium groups with silicon and its compounds.
- 15 The principal object of the invention is to generally improve upon the process for making acid-proof alloys to be used for casting chemical apparatus.

Another object is to adapt the process to the daily varying requirements of a foundry and to avoid the use of converters or open hearth furnaces and other equipments costly in installation and operation which have been hitherto used for such purpose, using 25 instead the simple and handy reverberatory furnace.

Another object of the invention is to save fuel and labor and to produce in a short time a homogeneous alloy of proper temperature 30 for casting, reducing the formation of slag to the least possible quantity.

Still another object is to produce by a simple process an alloy of predetermined composition which only contains a certain 35 low percentage of carbon and is almost free from undesirable foreign constituents.

In the processes hitherto employed in the manufacture of acid proof apparatus it was difficult to obtain castings which come out 40 faultless and do not crack when heated in use.

For the purpose of decreasing the very undesirable hardness of such alloys resulting from high percentage of silicon, iron poor in 45 carbon, such as wrought iron, soft iron, or steel scraps were used for making up the bulk of the charge, which means melting down large quantities of metal having a very high melting point.

50 It is obvious that the cupola of the foundry is not the proper equipment for this purpose; besides taking a long time to melt such charge down, a uniform reliable composition and purity of the alloy cannot be 55 obtained due to the influence of foreign matter with which the metal comes in con-

tact, while passing through the cupola. Also the crucible furnace does not come in question for practical manufacture of the large size castings used in the chemical industry. The electrical furnace, although being generally the ideal means for alloying iron is in most cases out of the question, due to the high cost of current. The open hearth furnace which of course is most appropriate 60 requires continuous operation and, besides being very expensive, cannot be adapted to the daily varying requirements of a foundry. The converter with the machinery connected therewith is also very expensive and 65 does not yield an alloy of reliable composition and quality, besides consuming considerable quantities of expensive material.

All these disadvantages are avoided by my new process which, in addition, yields an 70 alloy of reliable and uniform predetermined composition and just of the right pouring 75 temperature.

My invention makes it possible to use a simple reverberatory furnace which is the 80 cheapest furnace and very handy in many foundries, and to produce in such a furnace the silicon alloy which has the predetermined composition, is thoroughly homogeneous and has the proper temperature for 85 pouring, with the least possible consumption of fuel.

In using my new process for the making of the acid proof iron silicon alloy, the percentage of silicon in which varies according 90 to requirements from five to twenty-five per cent I heat a calculated charge of wrought iron, soft steel or the like together with the necessary amount of silicon, preferably in form of commercial ferro-silicon of a pre- 95 determined high content of silicon.

The components, iron and silicon, in lump form are dumped into the furnace in roughly intermixed state. The furnace is then heated from without in any suitable manner to a 100 temperature at which exothermic reaction is initiated in the charge, which will be at a temperature several 100 degrees C. below the fusing joint of the components at about 1250°, or roughly between 1200 and 105 1300° C. It suffices if at the stated temperature a piece of iron or the like and a piece of silicon are in contact, at which point of contact the reaction will then start with an abrupt rise in the temperature curve and 110 will then quickly, almost instantaneously, flash throughout the entire mass. In prac-

tical operation the entire charge of a large furnace, after the reaction temperature has been reached and reaction has set in at a single spot, will spontaneously melt down 5 within a few seconds. The reaction may also be started by prodding or striking the solid charge with an iron rod whereby local pressure between the more or less loosely contacting components is exerted. The re- 10 sult of this violent reaction is a complete liquefaction and the formation of a thoroughly homogeneous alloy, which readily separates from slag and other impurities, of which there will be very little at best 15 owing to the quickness and thoroughness of the conversion.

It will be understood that the process can be adapted, within the scope of the same invention, to the use of silicon in the 20 form of various silicon compounds and of almost pure silicon, either alone, or in mixture.

It will be further understood that the same invention may be used for alloying 25 other metals of the iron group such as manganese, nickel and cobalt, and also of metals of the chromium group, (chromium, tungsten, etc.) with silicon, the latter being preferably introduced in form of one of its com- 30 pounds such as ferro silicon, silicon-manganese, or the like, however, also pure or commercial silicon may be used alone or mixed with its compounds.

Since pure silicon is too expensive for use 35 on a large scale for industrial purposes, it will be found to answer the purpose to use high-per cent ferro-silicon (80-90%). With such percentage the exothermic reaction will proceed as set forth, and it will even take 40 place in the case of commercial 45% ferro-silicon, although in this latter instance it will not reach quite as high a temperature as in the case of the higher per cent material.

It is also to be understood that my method 45 is not confined to the use of a reverberatory furnace and that other kinds of flame heated furnace chambers may be adapted to my invention, provided that they can hold a bulky charge, are equipped with means to 50 raise the temperature to the reaction point and with a hearth for collecting and refining the alloy.

What I claim is:—

1. The process of alloying silicon with 55 metals of high melting point, which consists in heating a mixture of said components to a temperature at which exothermic reaction is initiated, and in then using this reaction to melt down the charge and complete the process.

2. The process of making alloys of metals

of the iron and chromium groups and silicon, which consists in heating the inter- 65 mixed components to a temperature at which exothermic reaction sets in, and in then using this reaction to melt down the charge and complete the process.

3. The process of making alloys of metals of the iron and chromium groups and silicon compounds of metals of said respective 70 groups, which consists in heating the inter- mixed components to a temperature at which exothermic reaction sets in, and in then using this reaction to melt down the charge and complete the process.

4. The process of making an acid proof 75 iron alloy consisting of heating a mixture of wrought iron, soft steel or the like with silicon until the chemical reaction between the silicon and the soft iron is initiated, 80 and of then using the heat of reaction for melting and finishing the alloy.

5. The process of making an acid proof 85 iron alloy consisting of heating a mixture of soft iron which is low in carbon with silicon in form of ferro silicon until the chemical reaction between the silicon and the soft iron is initiated, and then using the heat of reaction for melting and finishing 90 the alloy.

6. The process of making acid proof cast- 95 ings for chemical apparatus consisting of heating a charge of soft iron or steel mixed with ferro silicon in a flame heated furnace until the chemical reaction of the silicon upon the iron is initiated, and melting down the charge and finishing the alloy ready for pouring by the heat developed by the chemical reaction.

7. The process of making acid proof cast- 100 ings for chemical apparatus consisting of heating a charge of iron low in carbon mixed with ferro silicon in a reverberatory furnace until the chemical reaction of the silicon upon the soft iron is initiated, and melt- 105 ing down the charge and finishing the alloy ready for pouring by the heat developed by the chemical reaction between the iron and silicon.

8. The method of making acid proof cast- 110 ings for chemical apparatus consisting of heating a charge of soft iron low in carbon mixed with silicon in form of ferro silicon on a hearth in a furnace chamber to a tem- 115 perature of between 1200 and 1300 centi- grades for starting the chemical reaction between the iron and silicon and then melting down the charge and finishing the alloy ready for pouring by the heat spontaneously developed by said chemical reaction. 120

In testimony whereof I affix my signature.

RICHARD WALTER.